

Nov. 14, 1944.

R. M. BOEHM ET AL  
PROCESS OF PRODUCING CARBON AND ACTIVATING  
THE SAME, AND PRODUCTS THEREOF  
Filed March 16, 1940

2,362,463



INVENTORS  
ROBERT M. BOEHM  
HORACE E. HALL  
BY  
*Dyke & Schaefer*  
ATTORNEYS

Patented Nov. 14, 1944

2,362,463

# UNITED STATES PATENT OFFICE

2,362,463

## PROCESS OF PRODUCING CARBON AND ACTIVATING THE SAME, AND PRODUCTS THEREOF

Robert M. Boehm and Horace E. Hall, Laurel, Miss., assignors to Masonite Corporation, Laurel, Miss., a corporation of Delaware

Application March 16, 1940, Serial No. 324,442

6 Claims.

(Cl. 252—267)

Our invention relates to carbon and to a carbon base material for carbonizing, and to the process of manufacture thereof.

Our carbon base material and carbon can be made from hard fibrous vegetable materials such as wood of trees, or woody material of annual growths such as bamboo, cane, cornstalks, and the like, and nut and seed hulls containing lignocellulose in large proportions, as cottonseed hulls for example. Wood is the preferred material, and its use and treatment will be described in order to provide an illustrative embodiment affording an understanding of the invention.

With our invention, substantially the whole of the wood is used and there is no need for preliminary digestion and removal of parts thereof as in paper making for example.

Wood has heretofore been used in making carbon, as in the form of compressed briquettes of wood flour or compressed pieces of wood in natural state, but has the objection that swelling takes place particularly in drying briquettes made therefrom, even though the material such as wood flour be briquetted under very high pressure. While cracking and fissuring may not always be readily apparent upon swelling taking place at this stage, strains appear to be set up in the wood flour briquette which has swelled in drying, and to lead, upon carbonizing and other heat treatments, to formation of cracks, ruptures, and crumbling not permissible in high-grade carbon. It is an object of the present invention to eliminate objections of this nature by the preparation from wood of a material which in turn is carbonized to produce the carbon, and which material, occupying a status intermediate between the wood on the one hand, and the carbon on the other hand, and designated herein the "carbon base material," does not swell upon being dried, but on the contrary, shrinks in the course of its drying, and briquettes thereof for example are free from strains, cracks and fissures after drying, and do not crack or rupture upon carbonization, or upon roasting and activation, and yield high grade primary carbon and activated carbon of high density and hardness.

Heretofore in making compressed blocks or briquettes of various materials to be carbonized, binding materials such as sugars, tars and the like, have sometimes been added before briquetting to serve as a binder and to increase the density of the carbon made from the briquettes. One of the objects of our invention consists in eliminating need for such additions. With our invention added binders are not needed because our new carbon base material is self-bonding, or in other words contains bonding materials formed in the course of its production, including sugars, wood tars and the like. With a small moisture content as about 5-10%, it has substan-

tially plastic properties and can be compressed without added binder into strong, dense, self-bonded briquettes.

Resort has heretofore sometimes been had to carbonizing materials under pressure in order to make carbon of increased density and hardness. While we could carbonize our new carbon base material under pressure if desired, it is an object of our invention to eliminate need for carbonizing under pressure. There is no need for use of pressure in carbonization and other heat treatments of our carbon base material because the briquettes thereof, not only shrink in drying as stated, but continue to shrink extensively in carbonizing, etc., treatments, and yield strong dense hard carbon.

A further object consists in dispensing with need for use of dehydrating agents such as zinc chloride, for example, heretofore considered essential for production of high-grade carbon.

A further object consists in the provision of a novel type of high-grade primary carbon with a hardness over 120 on the Rockwell scale and a specific gravity over 1.1, and preferably over 1.2, and roasted and activated carbon of still higher hardness and specific gravity. The invention also includes other objects which will appear or be pointed out.

The first step of carbon manufacture is the making of the intermediate or carbon base material from the wood. In this step, the wood in somewhat subdivided state, preferably wood in the form of chips of approximately 1" maximum dimension, is subjected to high temperature and pressure in presence of moisture, and the temperature, pressure and time of such treatment is so regulated as to convert the ligno-cellulose material to a condition in which it will shrink upon drying and yield good high density carbon upon carbonization and subsequent heat treatments.

This treatment which we shall call thermo-hydrolysis is preferably effected with high pressure steam, and steam treatment will be described. When the steam treatment is terminated, the converted material is subdivided to a state of fineness. While the reduction to fineness can be performed separately, as by grinding after termination of the steam treatment, we preferably carry out the steam treatment by subjecting the chips to high pressure steam, as for example steam at a pressure of about 300-1200 lbs. per sq. in. or higher, and preferably at about 1000 lbs. per sq. in. in a gun or like apparatus, such as the gun disclosed in U. S. Patent to Mason No. 1,824,221 and consisting of a rugged upright cylindrical container equipped with a loading port at the top, a quick opening hydraulically operated discharge valve at the bottom and provided with a steam inlet,—and then terminate the steam treatment quickly and also

reduce the material to fineness by the disintegrating explosive discharge of the material from the region of high pressure in the gun chamber, which ensues upon the opening up of the outlet from the gun chamber to a region of much lower, preferably atmospheric, pressure.

(Treatment of wood with high temperature and pressure in presence of moisture is known and also the use of steam therefor and for thereafter causing disintegration by explosive discharge of the material is known in the prior art, and same are not claimed herein per se, but only the application thereof to the manufacture of carbon base material and carbon, which is new with us.)

The finely exploded carbon base material on dropping from the cyclone, or other separating device into which the discharge from the gun is preferably led, can be collected and used without adding water or washing. However, by reason of the wood sometimes containing initially a considerable proportion of water, as for example approximately 30%, and there being more or less condensation to water of the steam used for the heat and explosion treatment, the heat-treated and disintegrated carbon base material may contain a considerable proportion, as for example 50% of water, in which case partial drying can be resorted to in order to adjust the moisture content as may be desired.

With a given steam pressure, as for example 1000 lbs. per sq. in. and the steam treatment followed by explosive disintegration, the time of steam treatment required for the preparation of a carbon base material having the important properties of shrinking on drying from compressed state and upon carbonization, etc., heat treatments is to some extent dependent on the water content of the material used and on the nature of the material taken for treatment. This time is less for treatment of bone dry chips than for wet chips since conversion into steam of water in the chips will take extra time varying with the percentage of water contained in the chips. Hardwood requires longer treatment with steam than materials of annual growth, and pine wood requires somewhat longer steam-treatment than hardwood such as gumwood and the like. The treatment of gumwood, which is a type of hardwood and has an intermediate status from the standpoint of time of steam treatment required to secure the desired properties, will be selected to afford an exemplary disclosure.

In a preferred embodiment of the step of preparing the carbon base material as outlined above, fibrous ligno-cellulose material consisting of dry gumwood chips, was subjected to the action of steam at a pressure of 1000 lbs. per sq. in., and corresponding temperature of 285° C., the steam treatment consisting of first bringing the steam up to the pressure of 1000 lbs. per sq. in. in 30 seconds after the chips had been introduced into the gun and the gun closed, followed by holding the steam pressure of 1000 lbs. per sq. in. on the chips for 20 seconds. The steam-treatment was then terminated and the steam-treated material was thoroughly disintegrated by explosive discharge from the region of high steam pressure as above described. The resulting finely divided carbon base material, was substantially devoid of original fiber structure and substantially dough-like in consistency and dark in color. Briquettes made at a pressure of 10,000 lbs. per sq. in. from the material so produced and containing about 7% of moisture were found to

shrink about 5% upon drying to constant weight in four hours at 100° C. Good results were obtained by carbonizing this carbon base material, and good activated carbon obtained by roasting and activation of the primary carbon, and these treatments will be described later.

In making carbon base material good results can be secured by varying the time of holding at full steam pressure, as for example when using steam at 1000 lbs. per sq. in., varying the holding time from about 15 seconds to about 300 seconds. Lower steam pressure, such as 600 lbs. per sq. in. and corresponding temperature of 255° C. can be used by taking a longer time for the heat treatment, as about 1-10 minutes, and still lower pressures as down to about 300 lbs. per sq. in. with much longer times as about 15-40 minutes, but with somewhat less desirable results from the standpoint of explosive disintegration.

Higher pressures than 1000 lbs. as 1200 lbs. per sq. in. can also be used with shorter times as about 10-200 seconds.

Organic acids as acetic and formic acids are developed in the treatment with high pressure steam, and the carbon base material so produced in any of the ways above described is of low pH, usually below 3.5 pH. The acids appear to attack some parts of the wood fiber, and in any event, with exposure of the wood to steam at a pressure as high as 1000 lbs. per sq. in. for a holding time as long as 20 seconds for example, followed by explosion, the resulting carbon base material becomes substantially devoid of original fiber structure.

Sugars and the like may be incorporated with our carbon base material if desired, as heretofore sometimes practiced with other materials for carbonizing. However, with use of a starting material consisting of wood or equivalent lignocellulose material, and which contains hemi-celluloses and the like materials which are at least partially converted to sugar forming materials and sugars in the heat treatment process as above described, the addition of sugars from extraneous sources is ordinarily unnecessary. The sugar forming materials and sugars being freed or formed in situ in our carbon base material in the course of its production, and being retained therein, can perform the same functions in the carbonizing and other heat treatments, as if added from extraneous sources at resultant increased expense. Furthermore the sugars, etc., formed in the carbon base material itself are in a better state of distribution throughout the material than can be obtained by adding sugars from extraneous sources.

Constituents having bonding properties in addition to the sugars as above referred to, and apparently including wood tars, pentosans, hexosans, and the like materials, are also developed or freed by the steam treatment, and the steam-treated carbon base material is plastic or substantially so, and is self-bonding and so requires no added binder, although binders could be added if desired. This high self-bonding property of our carbon base material and its property of shrinkage without cracks and strains in drying from compressed state, and further shrinkage without rupture in carbonization and other heat treatments appear to be at least in large part a result of the steam treatment, since briquettes of wood material which have not been given such steam treatment, such as wood flour for example, even when compressed at 50,000 lbs. pressure per sq. in., swell upon drying and yield on carbonization

only a loosely bonded and crumbly carbon. The explosion treatment following steam treatment is also apparently beneficial in that gases and gas forming materials may be effectively swept out by the escaping steam.

We preferably form the preferably unwashed carbon base material into shapes. For example, the doughy material above referred to, with or without some adjustment of water content to get the most workable consistency, can be formed into ribbons by forcible extrusion through slot-like apertures, and dried in such ribbon form, and cut or broken into lengths before or after drying. While high density is not readily attainable by such extrusion, and for extrusion the water content must be fairly considerable, dried ribbons can be obtained which will yield carbon of fairly good strength and density.

In order to secure carbon of higher strength and density, the steam-treated and subdivided carbon base material is preferably formed into shapes of higher density than obtainable by such extrusion treatment, as for example it can be cold-compressed into blocks or the like shapes. For example, by adjusting the moisture content of the carbon base material prepared as above described to about 5%-10%, which can be accomplished by an expression treatment followed by partial drying, and then grinding the material and cold-compressing it under moderately high pressure, as 10,000 lbs. per sq. in., it can be inexpensively formed into blocks or briquettes which are of high density approaching the ultimate density of wood fiber, as for example, 1.35 sp. gr., and extremely hard. In these and other ways, dense, hard blocks can be made of practically any desired volume from quite large pieces to small pellets. Cold-compressing of the carbon base material at substantially room temperature is most desirable, as with this treatment primary carbon and activated carbon with higher density and hardness can be made from the resulting carbon base briquettes, pellets and the like than when this material is compressed in heated state and thereby cured to a vitreous-like state. It is of advantage particularly in making small pellets of the carbon base material to introduce a small percentage, as 0.1-0.5% for example, of lubricating material such as petrolatum, stearic acid or the like, and such material may be put into the gun with the chips if desired or may be added at a later stage.

The blocks, pellets or other shapes are thoroughly dried. When the carbon base material has been prepared by a steam treatment carried on for a desirably long time, as for example 20 seconds or more with steam at 1000 lbs. pressure per sq. in., and highly compressed, not only does no swelling take place during drying, but there is quite an appreciable shrinkage during the drying, as for example about 6% reduction in volume on reduction of the moisture content from approximately 7% to 0%. Weight reduction in drying is approximately in consonance with shrinkage in volume and no appreciable change in specific gravity takes place upon the drying of blocks or pellets of this carbon base material.

The drying can be effectively performed by heating to about 100° C. for a sufficient time, as about 4 hours with 1" blocks containing about 7% of moisture, and in this treatment, materials other than water which are volatile at this temperature, as some furfural and acetic acid for example, will be vaporized and driven off. The carbon base material is thus dried not only with complete absence of swelling but with definite

shrinkage, and with absence of cracks, and fissures, and of strains which would develop into such defects upon carbonization and later heat treatment. In pointing out below the extents

5 to which shrinkage or reduction in volume takes place upon subjection of our carbon base material to various heat-treatments, the volume of the dried blocks, pellets or the like before carbonization will be taken as the basis for comparison.

In the accompanying drawing forming a part of this specification the percentage of change in volume upon drying by drying in 4 hours at 100° C. the briquettes or pellets of our carbon base 15 material containing about 7% of moisture and compressed at a pressure of 10,000 lbs. per sq. in. is charted against the time in seconds at which these briquettes were made, dry gumwood chips 20 were held under 1000 lbs. steam pressure per sq. in. in the gun, following the bringing up to such pressure, and then explosively discharged.

As appears from this chart, with steam treatment holding time of about 3½ seconds at 1000 lbs. per sq. in. there is substantially no change 25 in the volume of the briquettes of carbon base material upon drying as above described. With a shorter time of exposure to such steam treatment in the gun, swelling of the resulting briquettes will take place upon drying, up to a maximum of about 8% in the case of exposure to the steam treatment for a period of 0 seconds, i. e., with the steam pressure merely brought up to 1000 lbs. per sq. in. and the charge immediately 30 exploded. Briquettes made of such materials given such short time treatment crack and rupture when carbonized and are not suitable for the purposes of our invention.

As the time of sustained exposure of the chips 40 to steam in the gun at this pressure is increased beyond about 3½ seconds, shrinkage will take place upon drying, and this shrinkage upon drying increases and approaches a maximum of about 6% with about 15 seconds' time of exposure of 45 the chips to such steam treatment in the gun, and the shrinkage upon drying remains about the same, namely about 6%, as the time of steam treatment of chips in the gun is further increased. A period of 20 seconds' exposure of chips in the gun to steam at 1000 lbs. per sq. in. is ample to ensure that the resulting carbon base material 50 will develop its maximum shrinkage on drying from compressed state, and yield good hard dense primary and activated carbon, and is therefore 55 preferred.

After drying, our new carbon base material is carbonized. The carbonization can be carried out without breaking up the blocks or pellets, but if desired, particularly when the pieces are 60 large, they can be cracked into relatively small pieces. The dry cracked material is preferably screened to desired minimum size which is used for carbonization, and the fines passing through the screen can be reground and reused in further making of block, ribbon, pellet or the like shapes, preferably admixed with fresh carbon base material.

Our carbon base material, which has been prepared in any of the ways above described as preferable, is believed to be unique in that, if desired, the carbonization can be rapidly performed on the material in relatively large pieces, as 1 inch or so in least dimension, without resulting cracking or rupturing, and with practically the same resulting density as when much longer time

is used in the carbonization treatment. For example, the carbonization of our carbon base material prepared by a steam treatment of chips at 1000 lbs. per sq. in. for 20 seconds as above described can be satisfactorily effected in three hours.

Carbonization over a period of 12-24 hours is, however, ordinarily preferable, particularly with large blocks, with a gradual heat increase up to about 450° C., care being exercised to prevent too rapid heat increase from exothermic causes. Air is excluded during carbonizing, the preferred atmosphere for this purpose consisting of CO<sub>2</sub> gas. Other inert gases can be used.

A further and very considerable shrinkage of previously dried and shrunk pellets, briquettes and the like made from our carbon base material takes place during carbonization, as a shrinkage to about one-half or somewhat less than one-half of the volume of the blocks, pellets, etc. in dry state prior to carbonization. The specific gravity is ordinarily reduced somewhat by the carbonization but this reduction is ordinarily not considerable, as for example a dry pellet of 1.35 sp. gr. may have its gravity reduced to about 1.1-1.26. The primary carbon so obtained is strong and hard and free from cracks, fissures and like defects. The apparent density of our primary carbon is approximately one-half the specific gravity, or about 0.55-0.63.

The carbon made from our improved carbon base material produced by sufficient exposure to steam treatment is very hard and resistant to abrasion. The following table shows in the right-hand column Rockwell hardness values of our primary carbons, and in the left-hand column shows the materials from which the carbon was produced.

Rockwell  
hardness  
number

Carbon made from wood flour briquettes  
compressed at a pressure of 50,000 lbs.  
per sq. in.

-97

Carbon made from gumwood chips converted to carbon base material under steam pressure brought up to 1000 lbs. per sq. in. and held at such pressure for times in seconds indicated below, and which are both above and below the preferable time, exploded from this pressure, and compressed with about 7% moisture content into briquettes at 10,000 lbs. per sq. in., and then carbonized for 14 hours at temperature to 450° C.:

|    |      |
|----|------|
| 0  | -67  |
| 2  | -45  |
| 5  | +16  |
| 8  | +76  |
| 10 | +123 |
| 12 | +125 |
| 15 | +128 |
| 20 | +128 |
| 30 | +128 |
| 45 | +128 |

It has been found that activation can be later carried on to best advantage and the densest activated carbon obtained when the primary carbon, obtained by carbonization treatment of our carbon base material as just described, is next given a roasting treatment. During roasting some of the residual hydrocarbons are driven off. This can be accomplished without appreciable loss of carbon by passing flue gas through the material,

but the oxygen content, if any, of the flue gas should be kept quite low, preferably under 5%. Carbon dioxide or inert gases such as nitrogen can be used. A desirable roasting procedure consists in application of a temperature of 750° C. for approximately 2 hours. Lower temperatures and longer times may be used, as approximately 600° C. for 4 hours. Additional shrinkage goes on during roasting, usually to approximately two-fifths of the volume of the blocks, pellets, etc., in dry state prior to carbonization, and takes place without cracking or the like. It is accompanied by some loss of weight caused by reduction in hydrocarbon content. The density is increased by the roasting, as for example pellets which had an apparent density of .55-.63, after carbonizing, may have this apparent density increased by roasting to about .65-.73.

The activation is next performed. During activation the remaining hydrocarbons are largely expelled, leaving activated carbon of enormous surface due to pores and capillaries having been emptied of hydrocarbon material.

While activation can be accomplished in various ways, the activation treatment which appears optimum for carbon made from our carbon base material, which has preferably first been roasted, consists of heating, in an atmosphere containing steam, to a temperature of approximately 850° C.-1000° C. for about 2 hours. In a preferred procedure, during the first hour a volume of superheated steam preferably equal to about one-half the weight of carbon is passed through it. During the second hour the volume of steam can be reduced, as to about one-fourth the weight of the carbon. A rotary kiln is preferably used for activation treatment in order to get uniform treatment throughout the material. Further shrinkage takes place during activation, bringing the volume down for example to approximately one-third of the volume in dry state prior to carbonization. The loss in density in activation, if any, is very slight, and in the activation treatment as in other heat treatments, a sound product is made free from fissures and cracks. The acidity of the carbon base material disappears in the heat treatments and the pH of the activated carbon for example is approximately 10.7.

The activated carbon so produced, when suitably ground and screened if made in large pieces, or without reduction in size if made in suitably small pellets, is suitable for use in gas masks, for absorption of vapors in industrial plants, and for purifying air in air conditioning systems, and various other purposes requiring a high-grade activated carbon. By making activated carbon out of small pellets of our carbon base material and with choice of proper size of the pellets, they can be made to shrink to predetermined size in drying, carbonizing, roasting, and activation, and used in gas masks and for solvent recovery for example, directly upon activation, without need for subdivision to smaller sizes. This activated carbon is very low in ash, a typical figure for ash content being 1.5%.

As has been indicated, the steps of steam-treatment and carbonization may overlap to some extent. Also while the steps of drying, carbonizing, roasting, and activating have been described separately and are preferably so performed, it is not essential that they shall be completely separate in all cases.

The use of dehydrating agents such as zinc chloride is not required with our invention at any

stage, and without their use a dense, hard carbon can be made by our invention which is at least the equal of the best grades of carbon produced with use of such agents. Elimination of need for such dehydrating agents is of great advantage since if used in preparing the carbon they must be washed out of the carbon for most applications, and this requires large quantities of water and subsequent drying. Dehydrating agents such as zinc chloride quickly destroy the effectiveness of copper or copper oxide customarily used in gas mask carbon, and if present in carbon to be used for solvent absorption and other commercial purposes they must be eliminated as completely as possible before the carbon can be used. In making our improved carbon no chlorides or equivalent materials need be added at any stage, and consequently no treatment is needed for their elimination, and in these and other ways our invention provides valuable high grade primary and activated carbon, and enables its production in large quantities from sources of material which are readily available, and at low cost.

From the material prepared from wood or equivalent ligno-cellulose material by use of high pressure steam as above described furfural and volatile organic acids may be recovered during drying and carbonization. By-products may also be obtained which are at least in part such as normally secured in connection with the destructive distillation of wood. The expressed liquors contain materials from which products such as furfural, organic acids as acetic and formic acids, sugars and sugar derivatives can be recovered. Still further by-product recovery can be accomplished by condensing the steam used for steam-treatment and explosion of the chips and carrying volatile constituents therefrom.

We claim:

1. Process for producing carbon material comprising the steps of providing a supply of loosely subdivided, fibrous, ligno-cellulose material, subjecting said material to steam at an elevated pressure for a sufficient time to eliminate substantially all original fiber structure, disintegrating such treated material into a mass of particles, partially drying the mass of particles in such manner and to such extent that the greater proportion of water is removed and most of the water soluble material formed during the heat treatment is retained therein, cold-compressing said particles, drying the material at such temperatures and for such a period of time as to cause material shrinkage and as to avoid any substantial occurrence of cracks and fissures therein on said drying and on further heating, and carbonizing the compressed material in the substantial absence of oxygen.

2. Process for producing carbon material comprising the steps of providing a supply of coarsely subdivided, fibrous, ligno-cellulose material, subjecting said material to steam at an elevated pressure for a sufficient time relative to the steam pressure employed to eliminate substantially all original fiber structure, disintegrating the material by explosive discharge from the region of

5 elevated steam pressure to a region of lower atmospheric pressure to form a mass of particles, said mass being of doughlike consistency, partially drying the mass in such manner and to such extent that the greater proportion of water is removed and most of the water soluble material formed during the heat treatment is retained therein, cold compressing a mass of said particles, drying the material at such temperatures and for such a period of time as to cause material shrinkage and as to avoid any substantial occurrence of cracks and fissures therein on said drying and on further heating, and carbonizing the compressed material in the substantial absence of oxygen.

10 3. Process for producing activated carbon which comprises the steps of providing a supply of coarsely subdivided, fibrous, ligno-cellulose material, subjecting said material to steam at an elevated pressure for a sufficient time to eliminate substantially all original fiber structure, disintegrating such material into a mass of particles, partially drying the mass of particles in such manner and to such extent that the greater proportion of water is removed and most of the water soluble material formed during the heat treatment is retained therein, cold compressing said particles, drying said compressed material at such temperatures and for such a period of time as to cause material shrinkage and as to avoid any substantial occurrence of cracks and fissures therein on said drying and on further heating, carbonizing the material by subjecting same to carbonizing temperatures in the substantial absence of oxygen, and subjecting the carbonized material to activating conditions.

15 4. Process for producing activated carbon which comprises the steps of providing a supply of coarsely subdivided, fibrous, ligno-cellulose material, subjecting said material to steam at an elevated pressure for a sufficient time relative to the pressure employed to eliminate substantially all original fiber structure, disintegrating the material by explosive discharge from the region of elevated steam pressure to a region of lower atmospheric pressure to form a mass of particles, said mass being of dough-like consistency, partially drying the mass in such manner and to such extent that the greater proportion of water is removed and most of the water soluble material formed during the heat treatment is retained therein, cold-compressing a mass of said particles, drying said compressed material at such temperatures and for such a period of time as to cause material shrinkage and as to avoid any substantial occurrence of cracks and fissures therein on said drying and on further heating, carbonizing the material by subjecting same to carbonizing temperatures in the substantial absence of oxygen, and subjecting the carbonized material to activating conditions.

20 5. A carbon material produced by the process defined in claim 1.

6. An activated carbon material produced by the process defined in claim 3.

ROBERT M. BOEHM.  
HORACE E. HALL.